

## UNITED STATES PATENT OFFICE

2,172,626

## MAGNETIC MATERIAL

Jacob Louis Snoek, Eindhoven, Netherlands, assignor to N. V. Philips' Gloeilampenfabrieken, Eindhoven, Netherlands

No Drawing. Application October 21, 1937, Serial No. 170,302. In Germany November 13, 1936

2 Claims. (Cl. 75—123)

My invention relates to magnetic material, and more particularly to a material which can be very readily powdered, and to magnetic cores and the like made from such powder.

To be suitable for the manufacture of powder or mass cores, a material must have the following main properties: (1) It must be very brittle so that it can be readily powdered, (2) it must have a low coercive force to insure low hysteresis losses.

According to the invention I obtain the above results by using an alloy consisting of from about 7 to 9% silicon, 6 to 11% manganese, and the remainder iron. Such alloys are very brittle and thus can be ground to a powder in a mill to obtain particles of the desired small size. Furthermore the coercive force of a solid piece of such material is very low as appears from the following table covering three alloys containing 8% of silicon, and 6, 8 and 10% respectively of manganese.

| Si      | Mn      | Fe      | Coercive force |
|---------|---------|---------|----------------|
| Percent | Percent | Percent | Oersteds       |
| 8       | 6       | 86      | 0.50           |
| 8       | 8       | 84      | 0.20           |
| 8       | 10      | 82      | 0.90           |

Furthermore, the electrical resistivity of the material according to the invention is relatively high, which results in low eddy current losses. For instance, an alloy containing 10% Mn and 8% Si and the remainder iron, has a resistivity of about  $1.5 \times 10^{-4}$  ohms per cubic centimeter.

The properties of the material can be further improved by annealing, after it has been powdered, at a high temperature of for instance 1100° C. for one hour. Due to such a heat treatment, which may be effected in an atmosphere of hydrogen or wet hydrogen the internal stresses present in the grains after the powdering operation are removed, so that a low coercive force is retained. Furthermore the material has the favorable property of hardly sintering at the above annealing temperature, whereas, impurities which affect the coercive force, such as carbon, are expelled from the material due to the annealing operation. After the above heat treatment an alloy containing 10% Mn, 8% Si, had a coercive force of about 0.08 Oersted. In making a magnetic core, the powdered material may be insulated in a suitable manner, for instance by coating the particles with a layer of zinc am-

monium phosphate, mixed with a binder. Subsequently the material is pressed into cores of the desired shape. Such cores have very low hysteresis and eddy current losses and thus are very advantageous in the manufacture of coils for high and low frequency purposes.

I first give a complete description of the manner of making a core for high frequency purposes.

82 parts (by weight) of commercial iron (containing about 0.03% C) with 10 parts of manganese and 8 parts of silicon are melted together in a high frequency furnace and poured out into coquilles in the form of large flat plates. These plates are taken from the coquilles when still very hot (about 1200° C.) and thrown into cold water.

After this the material is very easily crushed to particles measuring no more than 5 mm. in diameter. The latter are put into a steel ball mill through which a slow and continuous stream of dry air is passing thus causing the lightest particles formed during milling to leave the mill and settle down in a large glass container. The maximum size of the particles thus sieved out is about  $30\mu$ , as shown by the microscope, but the mean size is much smaller.

The powder is mixed with a concentrated ammoniacal solution of ammonium phosphate (about 10% by weight) from which the excess ammonia and the water is driven out at a temperature of about 80° C. After this the binder (6% by weight of a Bakelite resin) is added in the usual way.

The above mixture is pressed under a pressure of about 2 tons per sq. cm. into cylindrical cores having a diameter of 7 mm. and a length of 14 mm. The cores made in this way were investigated in a kind of Epstein arrangement (16 cores are put into a square, the corners being filled with suitable material) and the permeability  $\mu$  and eddy current loss measured between 200 and 600 meters. It was found that  $\mu=10.9$  and

$$c_f = \frac{R_e}{Lf^2} = 1.03 \times 10^{-8}$$

in which,

$c_f$  is the eddy current loss factor in ohms per henry per cycle,

$R_e$  is the equivalent eddy current loss resistance in ohms,

$L$  is the self-inductance of the Epstein arrangement in henries, and

$f$  is the frequency in cycles per sec.

For lower frequencies higher permeabilities are as a rule required. To that end the above mentioned process is slightly altered. Instead of using an open ball mill a mill is used, which is carefully closed, while the air content is driven out by CO<sub>2</sub>. After 12 hours milling the mill is opened and the content sieved out by blowing.

Powder material prepared in this way and otherwise similarly to the above mentioned method was pressed into a ring of square cross-section (thickness 1 cm. outer diameter 5 cm.) and investigated at 1800 cycles per sec.

The permeability was found to be 24, and the hysteresis factor C<sub>h</sub> in ohms per henry as obtained from the following formula was found to be 52.

$$C_h = \frac{R_h}{L\sqrt{L}} = 52$$

in which

C<sub>h</sub> is the hysteresis loss factor in ohms per henry, R<sub>h</sub> is the equivalent hysteresis loss resistance in ohms, and

L is the self-inductance in henries of the coil wound upon the core.

The eddy current losses at the above frequency were too small to be measured.

The ohmic resistance of the core mass varies 5 between 10<sup>5</sup> and 10<sup>7</sup> Ω per cubic centimeter, which is very useful in keeping extra losses due to capacitive currents through the iron core low.

While I have described my invention in connection with specific examples and applications, 10 I do not wish to be limited thereto but desire the appended claims to be construed as broadly as permissible in view of the prior art.

What I claim is:

1. A magnetic material for use in powder cores 15 and the like consisting of an alloy containing from 7% to 9% silicon, from 6% to 11% manganese and the remainder iron.
2. A magnetic material for use in powder cores 20 and the like consisting of an alloy containing about 8% silicon, from 6% to 11% manganese, and the remainder iron.

JACOB LOUIS SNOEK.